

# UNITED STATES PATENT OFFICE.

WILLIAM MARSHALL PAGE, OF CHESTER, PENNSYLVANIA.

## PROCESS OF UNITING COPPER TO FERROUS METALS.

1,171,066.

Specification of Letters Patent.

Patented Feb. 8, 1916.

No Drawing.

Application filed June 17, 1913. Serial No. 774,162.

*To all whom it may concern:*

Be it known that I, WILLIAM MARSHALL PAGE, a citizen of the United States, residing at Chester, in the county of Delaware and State of Pennsylvania, have invented certain new and useful Improvements in Processes of Uniting Copper to Ferrous Metals, of which the following is a specification.

10 This invention relates to processes of uniting copper to ferrous metals; and it comprises a process wherein a body of copper-iron alloy, of relatively low iron content is produced by the addition to molten copper, or to copper already containing iron, of suitable quantities of iron or steel in company with a deoxidizing agent such as phosphorus; a body of iron or steel is then brought into contact with the resulting 15 molten copper-iron alloy and is filmed or coated therewith, and a body of substantially pure copper is finally united to the alloy coating; all as more fully hereinafter described and as claimed.

20 25 In successful processes of uniting copper to steel or iron, the billet or other body of steel to be coated or clad is first brought into contact with copper heated considerably above its melting point to receive a preliminary film coating or linking layer to which a larger body of copper is subsequently united by casting or otherwise bringing copper at or near ordinary casting temperatures into contact with such preliminary film coating.

30 35 The temperature of the filming bath is such that, in spite of the fact that iron and copper do not have any marked tendency to unite integrally or weld together at temperatures around the melting point of copper, nevertheless at this higher or "super-molten" temperature a union between the copper and the iron or steel which is in the nature of, or equivalent to, a weld does take place. As a result, the preliminary film coat 40 45 or linking layer of copper or copper iron alloys is practically integral with the ferrous metal base to which it is attached. Union having been thus attained, it is found in practice a comparatively simple matter to weld-unite to the copper-surfaced billet or other body of ferrous metal a body of pure copper of any desired thickness, there being no difficulty in thus welding copper to copper. Copper applied at ordinary

50

casting temperatures merges readily with 55 the linking layer of copper-united by the first step of the process to the iron or steel. Methods of this general type and the products produced thereby are described and claimed in United States Patents 853,716 60 and 893,932 to John F. Monnot.

I have discovered that the production of the preliminary or film coat of copper on iron or steel is facilitated if the copper of the filming bath contains iron in rather small proportions. In other words, the union of copper with the ferrous metal base occurs more readily and certain other desirable advantages are secured, if a copper-iron alloy of low iron content be employed as the filming 65 bath, rather than ordinary copper. On account of this more ready union of iron with a copper-iron alloy than with ordinary copper, the temperature of the filming bath need not be so high as with such ordinary 70 copper. In my copending prior application Serial No. 556,601, filed April 20, 1910, this idea is disclosed broadly. As to such disclosure, the present application is a continuation of said prior application. 80

The present application has to do with improvements upon the process above described. The present process enables the ready production and accurate control in composition of copper-iron alloys of the 85 type desirable in the preliminary filming bath with which the iron or steel base is first brought into contact.

It is difficult under ordinary furnace conditions to alloy iron or steel and copper and to control the composition of the resulting bath. Solid iron does not dissolve readily in molten copper unless the copper bath be heated to temperatures approaching or exceeding the melting point of iron or of the 90 particularly steel employed. Furthermore, where the copper bath is heated directly by gas or oil firing as is customary in practice, it is practically impossible to avoid more or less pronounced oxidizing conditions in 95 attaining the temperatures necessary. In order to obtain efficient utilization of fuel and intense heat some excess air must be used. Under such conditions molten copper invariably contains some cuprous oxid. 100 When iron is added to such a body of molten copper, since iron has a greater affinity than copper for oxygen, there is preferential or 105

selective oxidation of the iron, part of the iron reducing the cuprous oxid with the formation of oxids of iron while the remainder is progressively oxidized by the furnace 5 gases as long as there is any iron left in the bath. Iron also has a purifying action in removing other impurities, such as sulfur, from the copper. Copper is apt to take up some sulfur from the furnace gases.

10 It is apparent therefore that the iron content of the bath is difficult to control and regulate under the conditions described. Such control and regulation are, however, of great importance where uniformity in 15 final product is required as in the production of copper-clad steel wire. The conductivity of such wire must be a maximum and must also be uniform for commercial application in telephone and telegraph lines and 20 in other electrical work. Relatively slight variations of the conditions prevailing in the process, particularly as regards the composition and temperature of the filming bath, affect the conductivity of the finished 25 wire profoundly. And while high quality and uniformity of product are necessary, in commercial practice rapidity and efficiency of work are of course as necessary.

Another disadvantage incident to excessive oxidation of the iron in the molten bath arises from the fact that when a billet is dipped into the bath, particles of iron oxids are apt to attach themselves to the surface of the billet, in spite of the fact 35 that their specific gravity is less than that of copper, and thus prevent actual contact of the alloy or filming bath with the billet at such points. Oxids of iron may also be formed in place by the oxidizing action of 40 cuprous oxid dissolved in the metal of the bath. As a consequence, imperfections may occur in the union of copper to steel in the finished billet, and these are exaggerated in the subsequent rolling and drawing operations.

It is clear from the foregoing that for several reasons it is of the greatest importance to regulate carefully the iron content of the alloy or filming bath and to prevent excessive oxidation of the iron. These 50 objects, as well as certain other advantages, are attained according to the present process by the use of a powerful deoxidizing agent such as phosphorus employed in conjunction with suitable additions of iron to the filming bath, in such manner that the iron content of said bath is brought to a certain approximately definite percentage and the composition of the bath is maintained substantially constant while a billet 55 of iron or steel is being immersed in the bath for a suitable period of time to receive the desired alloy or film coating against which is to be subsequently cast a relatively thick 60 layer of pure copper. In practice the iron

content of the bath should be relatively low. From 1 to 3 per cent. of iron is found advantageous, around 2 per cent. being best, though these limits are not rigid.

In carrying out the present process, any 70 suitable apparatus may be employed, but for producing the copper-iron alloy or mixture and giving a steel billet its preliminary or film coating, I prefer to use the type of tilting furnace described in my copending 75 application 516,253, filed September 4, 1909. This furnace comprises a melting hearth or chamber heated by direct oil or gas firing and a dipping chamber arranged at one side of the melting chamber and connected 80 therewith. When the furnace is in heating or melting position, the metal being treated is exposed to the oil or gas jets on the hearth and is melted or maintained molten. When the furnace is tilted into dipping 85 position, molten metal flows into the dipping chamber or pocket which is of a depth and width suitable to accommodate the molten metal coming from the hearth to form a deep body into which the billet may be 90 dipped. Assuming a furnace of this type to be employed, I will now describe a typical embodiment of the present process as actually carried out in practice. A suitable amount of copper, say 15 tons, is melted in 95 the heating chamber and the heating is continued until the molten copper is very fluid and lively. Sufficient iron or steel is added either at or prior to this time to give about 2 per cent. of iron in the molten mixture 100 after allowing for the necessary losses in melting down and dissolving the iron. The iron or steel may be added as such, or, conveniently, as copper clad steel scrap. The addition of material quantities of metals 105 which would remain in the alloy bath, other than iron and copper, should be avoided however as disadvantageous, since it is desired to obtain a copper-iron alloy or mixture which for practical purposes is substantially free of other elements. The iron need not be extremely pure of course, the quantities of the elements usually occurring as impurities or otherwise in the usual 110 commercial grades of iron and steel doing no material harm. During this melting down and dissolving operation, it is unnecessary to go to great lengths to prevent oxidation of the iron. The dissolved iron shields the copper from oxidation and in so 115 doing itself suffers oxidation in part; and a further portion is of course oxidized directly by the furnace gases. But this loss can be allowed for in adding the iron to the bath; and it is cheaper to operate in this way 120 than to use the amount of iron theoretically required to produce the desired molten mixture and add phosphorus to afford protection against loss by oxidation. The latter method may be employed but about the only 125

advantage it offers is that smaller quantities of iron oxids are formed in the bath. Such oxids as are formed by the addition of the iron rise to the surface and collect there as a scum; and this action is facilitated by the subsequent treatment of the bath as will appear later.

The desired composition of the alloy bath having been attained as above described, it is now necessary to free the body of the bath of any particles of iron oxids which may have become entangled mechanically below the surface of the bath, and to hold the composition of the alloy bath substantially constant during the succeeding billet-filming step. I accordingly add a powerful deoxidant which will dissolve in the metal bath and diffuse therethrough rapidly. Phosphorus offers the greatest advantages for this purpose in practice. In certain cases other deoxidants may be used, but to less advantage. The amount of phosphorus necessary to add to the bath at this time varies somewhat with the conditions and with the amount of oxids present. Enough phosphorus should be added to free the body of the bath from oxids and to afford a certain excess available for protecting the metals of the bath from further oxidation for the brief period of time during which the filming operation can be accomplished. One function of the phosphorus is therefore to act as a steadier for the composition of the bath and it does so at the expense of its own oxidation. As long as any free phosphorus remains in the bath, neither the iron nor the copper undergoes oxidation and the composition of the bath as regards these metals is constant.

The appearance of the scum or crust on the surface of the bath on tilting the furnace to expose the metal to the air for a minute or so affords a convenient indication as to whether or not sufficient phosphorus has been added. A dark or black slag is a favorable indication, while a yellowish crust shows the presence of too large quantities of oxids of iron and the necessity for adding more phosphorus. When the alloy bath is of the proper composition, a cast test piece shows a characteristic close grained silky fracture and is tough and hard to break.

The copper iron alloy bath having been brought to a definite composition, the furnace is tilted to cause the molten metal mixture to flow into the dipping pocket or chamber. The scum or slag of oxids, etc., floating on the surface of the bath is now skimmed off and a steel billet which has been previously prepared and superficially cleansed as by sand-blasting, pickling and washing, steaming, etc., is immersed in the bath and allowed to remain therein for a period of time depending somewhat on the size and temperature of the billet to be

dipped. Operating with the filming bath at approximately 2250° degrees F., or thereabout, with a 300 to 400 pound billet the period of immersion should be in the neighborhood of 2½ minutes.

70

For handling the prepared and cleansed billet prior to its immersion and after it is filmed, I prefer to use a bottomless casing closed at the top and provided with means for admitting a reducing atmosphere such as acetylene or producer gas to its interior, within which the billet may be inclosed and protected from the air. Means are provided for suspending the billet in the casing and for lowering it therefrom into the filming bath. The casing may serve also as the side walls of a mold, after the filming coat has been applied, into which the final or main layer of copper is cast around the filmed billet. A casing mold of this type is described in Patent 853,716. Still another form and one which I find even more convenient is disclosed in my copending application, Ser. No. 607,338, filed Feb. 8, 1911.

75

After the billet has remained in the alloy bath a sufficient length of time to acquire the desired copper-iron alloy film, it is withdrawn from the bath into the protecting casing, gas being fed into the casing continuously to maintain a reducing atmosphere bathing the filmed billet. The casing with the contained billet is then set on a mold bottom and sufficient pure copper, which has been melted in a separate furnace, is cast around the filmed billet. After the mold and its contents have cooled sufficiently, the mold sections are knocked apart and the clad billet is transported to soaking and re-heating furnaces preliminary to being rolled and drawn down into wire.

105

Work is facilitated by correlating the speed of operation with the sizes of billet and apparatus and their temperatures that at the moment of applying the second or cast-on coat, the exterior surface of the alloy film is still liquid or soft. In the meantime, the alloy bath having cooled somewhat during the filming operation, it is returned to the heating chamber by tilting the alloy furnace back into its original position. The alloy bath is again brought up to the proper temperature, the furnace is again tilted to cause the molten alloy mixture to flow back into the dipping pocket and the filming operation is performed on another billet as previously described.

110

In order to keep the composition of the alloy bath sufficiently constant and to insure the absence of an undue amount of oxids in the bath it is necessary to frequently replenish the bath with additions of iron and phosphorus. The heating of the alloy bath after the filming operation necessarily occasions more or less burning out of the iron. In practice it is often ad-

125

130

visible to so replenish the bath at intervals of 4 to 5 minutes. These intervals correspond approximately to the period of time which separates the filming of any two successive billets, and it is convenient to add a small amount of iron immediately after each filming operation and just before the alloy furnace is tilted back into heating position. With each addition of iron, it is necessary to add a small amount of phosphorus to act as before in the role of a shielding agent for the iron and a steadier for the bath composition. Operating with the amount of copper here assumed, I find that after each filming operation an addition of from 10 to 15 pounds of iron and from  $\frac{1}{2}$  to 1 pound of phosphorus serves to keep the alloy bath at the desired composition and in the proper condition.

Not only does the phosphorus act as above described, but it also greatly facilitates the solution of the added iron in the molten bath. As above stated, iron alone does not dissolve in copper with great ease, and especially where the temperature of the bath is not run up to an excessively high point. But when phosphorus and iron are brought together in the bath the solution of the iron takes place with great rapidity and a uniform distribution of the iron throughout the bath is readily effected, even where the temperature of the bath is not at the excessively high degree above noted. It is possible that this effect is due to the formation of iron phosphid which has a low melting point. This would explain the rapid solution of the iron in the copper, and the phosphorus is then left free to exercise its protective functions. Where copper clad scrap is used for the additions of iron, a greater weight of such scrap must of course be employed in order to introduce the desired amount of iron.

The ferrous metal body whose protection with copper is herein contemplated, while specifically hereinbefore referred to as a steel billet is of course not necessarily confined to steel *per se*. The terminology employed is intended to include iron and steel bodies of all kinds. The steel may be a simple carbon steel or it may be any of the so-called alloy steels containing varying proportions of nickel, chromium, vanadium and the like.

What I claim is:—

1. The process of uniting copper to steel which comprises preparing a bath of a molten alloy or mixture of copper and iron of approximately predetermined composition, contacting therewith a body of steel until said body acquires an adhering coating or film, removing said body of steel from contact with said bath, and uniting a body of substantially pure copper to the filmed steel body.

2. The process of uniting copper to steel which comprises preparing a bath of a molten alloy or mixture of copper and iron of approximately predetermined composition, the proportion of iron being relatively small, contacting therewith a body of steel until said body acquires an adhering coating or film, removing said body of steel from contact with said bath, and uniting a body of substantially pure copper to the filmed steel body. 70

3. The process of uniting copper to steel which comprises treating molten copper with iron under non-oxidizing conditions to obtain an alloy or mixture of copper and iron, contacting said alloy or mixture in molten condition with a solid body of steel and maintaining such contact until said steel body is coated or filmed with the alloy or mixture, terminating the contact of the steel body with the molten mixture, and thereafter uniting a body of substantially pure copper to the filmed steel body. 80

4. The process of uniting copper to steel which comprises treating molten copper with iron and a deoxidant to obtain a molten bath of a mixture or alloy of copper and iron, said mixture being low in iron, dipping a steel billet into said bath to produce an adherent coating of copper iron alloy on 90 said billet, removing the billet from the bath, and casting substantially pure copper against the filmed billet. 95

5. The process of uniting copper to steel which comprises treating molten copper with iron and phosphorus to obtain a molten bath of a mixture or alloy of copper and iron, said mixture being low in iron, dipping a steel billet into said bath to produce an adherent coating of copper iron 100 alloy on said billet, removing the billet from the bath and casting substantially pure copper against the filmed billet. 105

6. The process of uniting copper to steel which comprises treating molten copper with iron and phosphorus to obtain a molten alloy or mixture of copper and iron comprising approximately between 1 and 3 per cent. of iron, said mixture being low in iron, dipping a steel billet into said bath to produce an adherent coating of copper iron 110 alloy on said billet, removing the billet from the bath, and casting substantially pure copper against the filmed billet. 115

7. The process of uniting copper to steel which comprises preparing a molten bath of an alloy or mixture of copper and iron of approximately known composition, maintaining said molten bath at relatively very high and fairly constant temperature, correcting the composition of said bath by adding iron and phosphorus thereto, and dipping a body of steel thereinto to produce an alloy coating on said billet. 120 125

8. The process of uniting copper to steel 130

which comprises preparing a molten bath of an alloy or mixture of copper and iron of approximately known composition, maintaining said molten bath at relatively very high and fairly constant temperature, correcting the composition of said bath by adding iron and phosphorus thereto, dipping a body of steel thereinto to produce an alloy coating on said billet, and casting substantially pure copper against said billet.

9. In a process of coating metals, the method which comprises adding substantially pure iron and phosphorus to copper

under melting conditions to obtain a molten alloy or mixture of copper and iron and dipping a steel billet in said bath to produce an adherent coating of copper-iron alloy on said billet. 15

In testimony whereof, I affix my signature in the presence of two subscribing witnesses. 20

WILLIAM MARSHALL PAGE.

Witnesses:

J. HORACE WITSEL,  
T. G. BUSH, Jr.